

June 18, 1946.

J. J. DUNN

2,402,383

METHOD OF MAKING TUBING

Filed Aug. 23, 1943

2 Sheets-Sheet 1



INVENTOR:

JERRY JAY DUNN,

BY:  
*John E. Jackson*  
HIS ATTORNEY.

June 18, 1946.

J. J. DUNN

2,402,383

METHOD OF MAKING TUBING

Filed Aug. 23, 1943

2 Sheets-Sheet 2

*Straightening and Sizing Machine*

**FIG. 2.**

RECIRCULATING FURNACE

CONVEYOR

ROLLER TYPE COOLING TABLE

10



**FIG. 3.**

INVENTOR:

JERRY JAY DUNN,  
BY  
John E. Jackson  
HIS ATTORNEY.

## UNITED STATES PATENT OFFICE

2,402,383

## METHOD OF MAKING TUBING

Jerry Jay Dunn, Ellwood City, Pa., assignor to  
 National Tube Company, a corporation of New  
 Jersey

Application August 23, 1943, Serial No. 499,671

4 Claims. (CL 148—12)

1

This invention relates to a method for improving the physical properties of tubular material, particularly the resistance to collapse of oil country goods such as casing, tubing and drill pipe.

In Patent No. 2,293,938 to Dunn et al. there is disclosed a cold-worked and heat-treated tubular article having a high resistance to collapse by reason of its stress-strain curve characteristics. It is there stated that the predetermination of the proper relation of the value of unit stress at the beginning of permanent deformation and its value at yield strength are of extreme importance in obtaining a stress-strain curve having high collapse values. According to the disclosures thereof, the stress-strain curve of the material of the patented article is that in which the proportional limit is at least 75% of the yield strength and the yield strength at least 75% of the tensile strength. The "proportional limit" is therein defined as a test wherein that value is associated with a permanent deformation of .01%. The yield strength is the conventional .2% set value. These same values will be used herein.

I have discovered that conventional cold straightening operations have a harmful effect on collapse resistance and it is an object of my invention to provide a method of making tubing wherein the disadvantages of cold straightening operations are not present.

The foregoing and other objects will be more apparent after referring to the following description and attached drawings, in which:

Figures 1 and 2, combined, disclose a mill layout for carrying out the method of the invention; and

Figure 3 shows a roller type cooling table.

The tubular article of the present invention is made from a steel containing .15% to .50% carbon, .25% to 2.00% manganese, and .50% maximum silicon. Alloying elements which do not harden by precipitation (such as nickel, molybdenum in small amounts, chromium and vanadium), may be added to improve ductility. However, no alloying elements which harden upon precipitation (such as copper, nitrogen, tungsten and molybdenum in large amounts) should be employed since they will have an unfavorable effect on the stress-strain characteristics of the metal.

For the sake of illustration, the invention will be described in connection with a tube composed of steel of the following analysis:

|             | Per cent |
|-------------|----------|
| Carbon      | .40      |
| Manganese   | 1.30     |
| Silicon     | .22      |
| Sulphur     | .025     |
| Phosphorous | .030     |

The conventional practice of forming a tube is heating a billet to the desired temperature, pass-

2

ing the heated billet through first and second piercing mills, reheating the billet, passing it through a Hi-Mill, reelers, and the sizing machine 2, all of which are shown in Figures 1 and 2. The tube is then cooled on the cooling table 4 and subjected to the conventional cold straightening operation.

A representative tube formed of the above steel by this conventional seamless tube practice, if allowed to cool to room temperature after being reeled and sized, has the following physical characteristics:

|                    |                  |         |
|--------------------|------------------|---------|
| Tensile strength   | lbs. per sq. in. | 108,000 |
| Yield strength     | do               | 63,000  |
| Proportional limit | do               | 60,000  |
| Elongation in 2"   | percent          | 26.8    |
| Collapse pressure  | lbs. per sq. in. | 4,850   |

I have discovered that a tubular article having the desired physical characteristics can be obtained by a final finishing step in which the diameter of the tubular article is reduced at least 3% and preferably between 6 and 10% while at a temperature between the so-called blue-heat zone and somewhat below the lower critical temperature of the steel of which it is composed, preferably between 650° and 1000° for conventional grades of oil well casing steel. A temperature of about 850° has been found to give good results.

Therefore, in accordance with the teachings of the present invention, the tube which is made about 8% oversize by conventional practice instead of being allowed to cool to room temperature after sizing, followed by a conventional cold straightening operation, is inserted after sizing in the recirculating furnace 6 and the temperature thereof equalized at a point between 650° and 1000° F., preferably at about 850° F. Following such equalization of temperature the tube is withdrawn from the furnace and quickly passed through a multi-stand set of sizing mill rolls 8 which are adjusted to reduce the diameter thereof about 8% and at the same time to straighten the tube. Upon emergence from the sinking or sizing mill 8, the tube is placed on a "roller" type cooling table 10 where it is rotated between successive "steps" thereover until it is sufficiently cooled to be placed upon a conventional cooling table without danger of uneven cooling, which causes out of roundness or warping. The temperature should be below 400° F.

The roller type cooling table 10 consists of rolls 12 which are rotated by any suitable means (not shown) and support the tube X as shown in Figure 3. These rolls keep the tube rotating while well supported along a straight line and therefore insure uniform cooling and maintain the tube straight. The tube is moved from one pair of rolls 12 to the next by means of indexing chain

## 3

13 which consists of links 14 supporting fingers 16. The sprocket wheel 18 is rotated, preferably intermittently, by any suitable means (not shown), and, in rotating, causes the fingers 15 on the chain to contact the tube X and move it to the next pair of rolls.

The tube which now has the same diameter and wall thickness as the conventional tube of the above tabulation is found to have the following improved physical properties:

|                    |                  |         |
|--------------------|------------------|---------|
| Tensile strength   | lbs. per sq. in. | 117,200 |
| Yield strength     | do               | 103,200 |
| Proportional limit | do               | 96,500  |
| Elongation in 2"   | per cent         | 18.5    |
| Collapse pressure  | lbs. per sq. in. | 6700    |

This increase in collapse pressure results in an increase of approximately 38% in the depths to which the treated casing can be set with a given factor of safety, permitting a weight savings of approximately 25%. These amounts will vary somewhat according to the steel composition and temperature and amount of cold work, but in all cases the treatment should result in at least a 20% increase in setting depths.

While one embodiment of the invention has been shown and described, it will be apparent that other modifications and adaptations may be made without departing from the scope of the following claims.

I claim:

1. A method of enhancing the physical properties and resistance to collapse of pipe composed of steel containing between .15 and .50% carbon, .50 to 2.00% manganese, and .05 to .50% silicon comprising forming a pipe of said steel having a diameter of at least 3% larger than that desired in the final product, equalizing the temperature of said pipe at a point between 650° and 1000° F., and reducing the diameter of said pipe while

40

5 at said temperature to that desired in the final product.

2. A method of enhancing the physical properties and resistance to collapse of pipe composed of steel containing between .15 and .50% carbon, .50 to 2.00% manganese and .05 to .50% silicon comprising forming a pipe of said steel having a diameter at least 3% larger than that desired in the final product equalizing the temperature of said pipe at a point between 650° and 1000° F., straightening and reducing the diameter of said pipe to that desired in the final product while at said temperature and maintaining the pipe in straight condition while cooling.

10 3. A method of manufacturing seamless pipe, having enhanced physical properties and high resistance to collapse, composed of steel containing between .15 and .50% carbon and .50 to 1.75% manganese, which includes piercing a solid billet and performing tube rolling operations thereon to obtain a reeled and sized work-piece of a slightly smaller wall thickness and a diameter at least 3% larger than that desired in the final product, equalizing the temperature of said reeled and sized work-piece at a point between 650° and 1000° F. reducing the diameter to that desired and straightening same while at said temperature and maintaining said pipe in a straight condition while cooling.

20 4. A method of enhancing the physical properties and resistance to collapse of pipe composed of steel containing between .15 and .50% carbon and .50 to 2.00% manganese comprising forming a pipe of said steel having a diameter at least 3% larger than that desired in the final product, equalizing the temperature of said pipe at a point between 650° and 1000° F. and reducing the diameter of said pipe while at said temperature to that desired in the final product.

JERRY JAY DUNN.